

# United States Patent [19]

Inoue et al.

[11] 3,793,098

[45] Feb. 19, 1974

[54] COMPOSITE DOUBLE BASE PROPELLANT  
WITH  $\beta$ -DIKETONE STABILIZER

[75] Inventors: Kazuhiro Inoue, Chita-gun;  
Kazutoshi Kito, Nagoya; Fumio  
Matsui, Chita-gun, all of Japan

[73] Assignee: Nippon Oils and Fats Company  
Limited, Tokyo, Japan

[22] Filed: Dec. 21, 1972

[21] Appl. No.: 317,122

[30] Foreign Application Priority Data

Dec. 27, 1971 Japan ..... 46/2635

[52] U.S. Cl. .... 149/19.8, 149/20, 149/38,  
149/98

[51] Int. Cl. .... C06d 5/06

[58] Field of Search .... 149/38, 98, 100, 50, 65, 76,  
149/79, 18, 19, 20

[56] References Cited

UNITED STATES PATENTS

3,711,344 1/1973 Pierce ..... 149/38 X

3,245,849 4/1966 Klager et al. .... 149/19  
2,982,638 5/1961 Cooley et al. .... 149/98  
3,228,815 1/1966 Henry et al. .... 149/98  
3,689,331 9/1972 Pierce ..... 149/98 X

Primary Examiner—Carl D. Quarforth

Assistant Examiner—E. A. Miller

Attorney, Agent, or Firm—Stevens, Davis, Miller &  
Mosher

[57] ABSTRACT

Propellant composition having an excellent stability at  
a high temperature is a composite modified double  
base propellant containing an oxidizing agent and a  
diketone having the general formula



wherein  $R_2$  and  $R_3$  are alkyl having one to 10 carbon  
atoms, haloalkyl having one to 10 carbon atoms or  
aryl radical.

3 Claims, No Drawings

**COMPOSITE DOUBLE BASE PROPELLANT WITH  
β-DIKETONE STABILIZER**

The present invention relates to a composite modified double base propellant composition having a high stability at a high temperature.

The present invention can provide a propellant composition having an extremely higher stability at a high temperature of 60° C than a conventional propellant composition, which is obtained by adding an  $\beta$ -diketone compound in the production of composite modified double base propellant (abbreviated as CMDB propellant hereinafter).

In general, CMDB propellant contains nitric acid esters, such as nitroglycerine, nitrocellulose and the like and an oxidizing agent, such as ammonium, potassium or lithium perchlorate or ammonium, potassium or lithium nitrate and therefore a small amount of water in the propellant dissolves the oxidizing agent and further promotes the decomposition of the nitric acid ester. This phenomenon is slow at room temperature but when the temperature is raised as an acceleration test for storage for a long period of time, the reaction may proceed rapidly to cause a foaming phenomenon. Such a propellant causes an abnormal combustion upon the combustion, which is a great demerit as the propellant.

5

compounds having the following formula are effective.



In the above formula,  $\text{R}_2$  and  $\text{R}_3$  are alkyl having one to 10 carbon atoms, haloalkyl having one to 10 carbon atoms or aryl radicals.

These compounds have been always used together with an isocyanate compound as an additive for prolonging the pot life of the polyurethane propellant.

However, the present invention has no relation to such an activity and it has been found that the foaming can be prevented by using the above described  $\beta$ -diketone alone.

The amount to be added varies in ammonium perchlorate series CMDB propellant and ammonium nitrate series CMDB propellant respectively but 0.5 to 2 percent by weight is preferable.

20 Namely, when the water content in the propellant is about 0.3 percent, if the amount is less than 0.5 percent, the foaming probably occurs and when the amount is more than 2 percent, it is not practicable in view of physical properties and property of combustion. However, the amount is not particularly limited.

25 The following examples are given for the purpose of illustration of this invention and are not intended as limitations thereof.

**EXAMPLES**

| Component                          | Example                                       | Comparative sample |    |    |    |     |    |    |    |    |    |
|------------------------------------|-----------------------------------------------|--------------------|----|----|----|-----|----|----|----|----|----|
|                                    |                                               | 1                  | 2  | 3  | 4  | 5   | 6  | 7  | 8  | 9  | 10 |
|                                    | Nitrocellulose.....                           | 20                 | 20 | 20 | 20 | 20  | 20 | 20 | 20 | 20 | 20 |
|                                    | Nitroglycerine.....                           | 37                 | 37 | 37 | 37 | 37  | 37 | 37 | 37 | 37 | 37 |
|                                    | Plasticizer.....                              | 9                  | 9  | 9  | 9  | 9   | 9  | 9  | 9  | 9  | 9  |
|                                    | Aluminum.....                                 | 16                 | 16 | 16 | 16 | 16  | 16 | 16 | 16 | 16 | 16 |
|                                    | Ammonium perchlorate.....                     | 18                 | 0  | 18 | 0  | 18  | 0  | 0  | 18 | 18 | 18 |
|                                    | Ammonium nitrate.....                         | 0                  | 18 | 0  | 18 | 0   | 18 | 0  | 0  | 0  | 0  |
|                                    | Potassium perchlorate.....                    | 0                  | 0  | 0  | 0  | 0   | 0  | 18 | 0  | 0  | 0  |
| Composition.....                   | Acetylacetone.....                            | 0                  | 0  | 1  | 0  | 0   | 0  | 0  | 0  | 0  | 0  |
|                                    | Benzoylacetone.....                           | 0                  | 0  | 0  | 2  | 0   | 1  | 1  | 0  | 0  | 0  |
|                                    | Propionylacetone.....                         | 0                  | 0  | 0  | 0  | 1.5 | 0  | 0  | 0  | 0  | 0  |
|                                    | <i>o</i> -Hydroxybenzoylpropionylmethane..... | 0                  | 0  | 0  | 0  | 0   | 0  | 0  | 1  | 0  | 0  |
|                                    | Benzoyl- <i>n</i> -butyroylmethane.....       | 0                  | 0  | 0  | 0  | 0   | 0  | 0  | 1  | 0  | 0  |
|                                    | Propionylisovalerylmethane.....               | 0                  | 0  | 0  | 0  | 0   | 0  | 0  | 0  | 1  | 0  |
|                                    | Chlorobenzoylacetoylmethane.....              | 0                  | 0  | 0  | 0  | 0   | 0  | 0  | 0  | 0  | 1  |
|                                    | Benzoyldichloroacetoylmethane.....            | 0                  | 0  | 0  | 0  | 0   | 0  | 0  | 0  | 0  | 1  |
|                                    |                                               | 6                  | x  | x  | o  | o   | o  | o  | o  | o  | o  |
|                                    |                                               | 12                 | x  | x  | o  | o   | o  | o  | o  | o  | o  |
|                                    |                                               | 18                 | x  | x  | o  | o   | o  | o  | o  | o  | o  |
|                                    |                                               | 24                 | x  | x  | o  | o   | o  | o  | o  | o  | o  |
| X-ray test..... Lapse of days..... | 30                                            | x                  | x  | o  | o  | o   | o  | o  | o  | o  | o  |
|                                    |                                               | 36                 | x  | x  | o  | o   | o  | o  | o  | o  | o  |
|                                    |                                               | 42                 | x  | x  | o  | o   | o  | o  | o  | o  | o  |
|                                    |                                               | 48                 | x  | x  | o  | o   | o  | o  | o  | o  | o  |
|                                    |                                               | 54                 | x  | x  | o  | o   | o  | o  | o  | o  | o  |

**Note:**

Numerical value: Weight percent.

In X-ray test, the formation of foam in propellant was determined.

x: Foam is formed. o: No foam.

60Φ x 100/ of hard vinyl chloride pipe was used and the upper and lower ends were sealed by a rubber.

Test temperature: 60°C.

The amount of the diketone added in the above Table shows the part by weight based on 100 parts of the composite modified double base propellant containing an oxidizing agent.

In order to solve such an inconvenience, it is necessary to restrain the foaming and the inventors have studied 65 concerning the foaming and found that  $\beta$ -diketone

What is claimed is:

1. A propellant composition having excellent high temperature stability comprising

a composite modified double base propellant consisting essentially of nitrocellulose, nitroglycerine and an oxidizing agent, having added thereto diketone of the general formula



wherein  $R_2$  and  $R_3$  are alkyl having one to 10 carbon atoms, haloalkyl having one to 10 carbon atoms or aryl radicals.

2. Propellant as claimed in claim 1, wherein said diketone is selected from the group consisting of acetylacetone, benzoylacetone, propionylacetone,  $\alpha$ -hydrobenzoylpropionylmethane, benzoyl-n-butyroylmethane, propionylisovalerylmethane, chlorobenzoylacetoylmethane and benzoyldichloroacetoylmethane.

3. Propellant as claimed in claim 1, wherein said oxidizing agent is selected from the group consisting of perchlorates and nitrates.

\* \* \* \* \*

15

20

25

30

35

40

45

50

55

60

65

UNITED STATES PATENT OFFICE  
CERTIFICATE OF CORRECTION

Patent No. 3,793,098 Dated February 19, 1974

Inventor(s) Kazuhiko INOUE et al

It is certified that error appears in the above-identified patent  
and that said Letters Patent are hereby corrected as shown below:

IN THE TABLE, numerals 6 - 54 should be included in the  
column of "Lapse of days" and "x" mark and "o" mark should  
be shifted to succeeding left columns respectively as  
shown in red by the attached Table.

Signed and sealed this 4th day of February 1975.

(SEAL)

Attest:

McCoy M. GIBSON JR.  
Attesting Officer

C. MARSHALL DANN  
Commissioner of Patents